

2,756,213

## AMATE-DICARBOXYLATE-THICKENED GREASE

Joseph A. Dixon, Berkeley, Calif., assignor to California Research Corporation, San Francisco, Calif., a corporation of Delaware

No Drawing. Application August 19, 1952,  
Serial No. 305,288

6 Claims. (Cl. 252—33.6)

This patent application is directed to new grease-thickening agents for high temperature grease compositions; that is, high temperature grease compositions thickened with amic acid salt-dibasic acid salt mixtures.

It is becoming more and more apparent that, for the most part, greases must be able to lubricate effectively under conditions of high temperatures, that is, temperatures considerably in excess of 400° F., and, in certain instances, in the range of 500° F. Numerous military and industrial grease specifications describe greases having dropping points of 400° F. as a minimum. This need for high temperature greases is the result of increased speeds of gears, bearings, and other moving parts; increased pressures caused by the development of smaller gears to withstand greater loads than heretofore expected of larger gears, etc.

In the automotive industry, for example, there is the constant desire to manufacture smaller internal combustion engines without sacrificing power output. In fact, many of these smaller engines are designed to deliver greater power than their larger counterparts. The same smaller engines have considerably less bearing surfaces than the larger predecessors, which means that the bearings gear greater loads than before.

Similarly, the continuing trend to manufacture automobiles with lower centers of gravity has made it necessary to use smaller gears, particularly in such gear assemblies as the differentials and transmissions. The smaller gears thus used have considerably greater pressures exerted upon them per unit area than the older type gear assemblies. Thus, machines having higher loads on bearings and gears along with greater speeds, require grease compositions which will function at higher temperatures than heretofore necessary.

Greases prepared according to the present invention will maintain grease consistencies at extremely high temperatures; that is, such greases will remain unctuous and not become hard or brittle at such high temperatures in the range of 500° F. Such greases also have excellent resistance to emulsion in water and have excellent anti-wear properties.

Certain amic acid salts of themselves thicken lubricating oils to the consistency of greases. Such amic acid salt thickening agents have been prepared from amic acids obtained by reacting stoichiometric amounts of amines and dibasic acids; that is, 1 mole of a primary amine (e. g., lauryl amine) was reacted with 1 mole of a dibasic acid (e. g., sebacic acid) to form the desired amic acid (e. g., N-monolauryl sebacamic acid). This amic acid was then reacted with a metal hydroxide (e. g., sodium hydroxide) to form the sodium soap of the amic acid (e. g., N-lauryl-sodium sebacamate) which was used as a grease thickening agent. Such amic acid salts of themselves are used in the preparation of greases having dropping points in the region of 400° F. However, they are ineffective in the preparation of greases having dropping points in the region of 500° F.

Dibasic acid salts (e. g., sodium sebacate) of them-

selves exhibit no gelation effect when heated in lubricating oils. That is, when dibasic acid soaps are mixed with lubricating oils, and such mixtures are heated to high temperatures (e. g., 500° F.), cooled, and milled, no gel structure nor grease is obtained.

However, it has been discovered that greases having extremely high dropping points, i. e., dropping points in the region of 500° F., can be obtained by the use of grease thickening agents set forth according to the present invention. These new high-temperature grease thickening agents comprise mixtures of amic acid salts and dicarboxylic acid salts. Thus, the grease compositions of the present invention comprise lubricating oils thickened with amic acid salt-dibasic acid salt mixtures.

The amic acid salt-dibasic acid salt mixtures of this invention are prepared by reacting 1 mol of a primary (or secondary) amine with at least 1.5 mols of a dibasic acid to form an amic acid-dibasic acid mixture; which mixture is then reacted with a metal oxide or hydroxide, resulting in an amic acid salt-dibasic acid salt mixture of the present invention.

The amic acid salts which are present in the grease thickening composition described herein are represented by the following formula



wherein R is a saturated or unsaturated, straight-chained, branch-chained or cyclic essentially hydrocarbonaceous radical having from 2 to 50 carbon atoms (8 to 20 preferred), R<sub>1</sub> is a saturated or unsaturated straight-chained, branch-chained, or cyclic essentially hydrocarbonaceous radical having from 1 to 54 carbon atoms, M is a metal, and x is a number having a value equal to the valence of the metal M.

It is preferred that R be a straight-chained or cyclic essentially hydrocarbonaceous radical and that R<sub>1</sub> be a straight-chained essentially hydrocarbonaceous radical.

Examples of the R radicals include the following: ethyl, propyl, propenyl, butyl, butenyl, pentyl, hexyl, hexenyl, octyl, octenyl, nonyl, decyl, decenyl, dodecyl, dodecenyl, tetradecyl, tetradecenyl, hexadecyl, octadecyl, octadecenyl, eicosyl, triacontyl radicals, radicals derived from petroleum hydrocarbons, such as white oil, wax, olefin polymers, e. g., polypropylene and polybutene, etc.

Examples of R<sub>1</sub> radicals include the following: methylene radicals, i. e., (CH<sub>2</sub>)<sub>x</sub>, wherein x is a number from 1 to 52 (6 to 24 preferred, 12 to 18 especially preferred) (including methylene radicals which may have one or more saturated or unsaturated, straight-chained, branch-chained, or cyclic essentially hydrocarbonaceous radical attached thereto); a phenyl radical; a substituted phenyl radical (wherein the phenyl nucleus contains one or more aliphatic radicals attached thereto); etc.

By "essentially hydrocarbonaceous" radicals is meant those radicals which are composed mainly of hydrogen and carbon and include such radicals which include, in addition, minor amounts of the substituents such as chlorine, bromine, oxygen, nitrogen, etc.

The dibasic acid salts present in the grease thickening mixtures of the present invention include those represented by the following formula:



wherein M represents a metal, x is a number having a value equal to the valence of the metal, and R<sub>2</sub> is a saturated or unsaturated, straight-chained, branch-chained or cyclic essentially hydrocarbonaceous radical; for example, a methylene radical, i. e., (CH<sub>2</sub>)<sub>x</sub>, wherein x is a number from 1 to 52 (4 to 16 preferred, 4 to 10 es-

pecially preferred) (including such methylene groups which may have one or more saturated or unsaturated, straight-chained, branch-chained or cyclic essentially hydrocarbonaceous radicals attached thereto); a phenyl group; a substituted phenyl radical (wherein the phenyl nucleus has one or more aliphatic radicals attached thereto); etc.

For sake of brevity, the "amic acid salts" will herein-after be termed "amates," and the "dibasic acid salts" will be termed "dicarboxylates."

The metals which can be used in the formation of the soaps of this invention include the metals of groups I, II, III, and IV of Mendeleff's Periodic Table. Particular metals include lithium, sodium, potassium, silver magnesium, calcium, zinc, strontium, cadmium, barium, aluminum and lead.

Lubricating oils which are suitable base oils for the grease compositions of this invention include a wide variety of lubricating oils, such as naphthenic base, paraffin base, and mixed base, other hydrocarbon lubricants, e. g. lubricating oils derived from coal products, and synthetic oils, e. g., alkylene polymers (such as polymers of propylene, butylene, etc., and mixtures thereof), alkylene oxide type polymers, dicarboxylic acid esters, liquid esters of acids of phosphorus, alkyl benzene polymers, polymers of silicon, etc. Synthetic oils of the alkylene oxide type polymers which may be used include those exemplified by the alkylene oxide polymers (e. g., propylene oxide polymers) and derivatives, including alkylene oxide polymers prepared by polymerizing the alkylene oxides, e. g., propylene oxide, in the presence of water or alcohols, e. g., ethyl alcohol; esters of ethylene oxide type polymers, e. g., acetylated propylene oxide polymers prepared by acetylating propylene oxide polymers containing hydroxyl groups; polyethers prepared from the alkaline glycols, e. g., ethylene glycol, etc.

The polymeric products prepared from the various alkylene oxides and alkylene glycols may be polyoxalkylenediols or polyalkylene glycol derivatives; that is, the terminal hydroxy group can remain as such, or one or both of the terminal hydroxyl groups can be removed during the polymerization reaction by esterification or etherification.

Synthetic oils of the dicarboxylic acid ester type include those which are prepared by esterifying such dicarboxylic acids as adipic acid, azaleic acid, suberic acid, sebacic acid, alkenyl succinic acid, fumaric acid, maleic acid, etc. with alcohols such as butyl alcohol, hexyl alcohol, 2-ethyl-hexyl alcohol, dodecyl alcohol, etc. Examples of dicarboxylic acid ester synthetic oils include dibutyl adipate, dihexyl adipate, di-2-ethylhexyl sebacate, di-n-hexyl fumaric polymer.

Synthetic oils of the alkyl benzene type include those which are prepared by alkylating benzene (e. g., dodecyl benzene, tetradecyl benzene, etc.).

Synthetic oils of the type of liquid esters of acids of phosphorus include the esters of phosphoric acid, e. g., tricresyl phosphate; the esters of phosphonic acid, e. g., the diethyl ester of decanephosphonic acid, etc.

Synthetic oils of the type of polymers of silicon include the liquid esters of silicon and the polysiloxanes. The liquid esters of silicon and the polysiloxanes include those exemplified by tetraethylsilicate, tetraisopropyl silicate, tetra (methyl-2-butyl) silicate, tetra (4-methyl-2-penta) silicate, tetra (1-methoxy-2-propyl) silicate, hexyl (4-methyl - 2 - pentoxy) disiloxane, poly(methylsiloxane), poly(methylphenylsiloxane), etc.

The above base oils may be used individually as such, or in various combinations, wherever miscible or whenever made so by the use of mutual solvents.

Examples of primary amines useful in the preparation of the thickening agents herein include ethylamine, propylamine, butylamine, butenylamine, pentylamine, octylamine, octenylamine, decylamine, dodecylamine, hexa-

mine, triacontylamine, etc. The amines may be used individually as such or as mixtures of amines.

Mixtures of amines used in the preparation of the thickening agents of this invention also include mixtures containing minor amounts (less than 50%) of secondary amines.

Examples of dicarboxylic acids include malonic acid, isosuccinic acid, methyl succinic acid, glutaric acid, adipic acid, pimelic acid, suberic acid, sebacic acid, dicarboxylic acids prepared by polymerizing unsaturated monobasic acids and derivatives (e. g., heating the methyl esters of linoleic acid to form a dilinoleic acid), etc. The dicarboxylic acids may be used either individually as such or as mixtures.

15 In the preparation of certain grease thickening agents herein, dicarboxylic acids were used which had been prepared by polymerizing unsaturated monobasic acids. These dicarboxylic acid preparations are known as Dimer acids, and they are obtained from Emery Industries, Inc., 10 Cincinnati, Ohio. These dicarboxylic acid preparations contain a small amount of tricarboxylic acids (approximately 12%), which also form grease-thickening agents when reacted with primary amines, followed by reaction with a metal oxide or hydroxide to form the amate-dicarboxylate-tricarboxylate grease-thickening agent.

20 As noted hereinabove, the amate-dicarboxylate mixture thickening agents of this invention are prepared by first reacting a primary amine with a dibasic acid in such proportions that the mol ratio of the dibasic acid to the amine has a value from 1.5 to 5.0, preferably from 2 to 4. This reaction produces a mixture of amic acids and unreacted dibasic acids, which mixture is then reacted with a metal oxide or hydroxide to form the desired mixture of amates and dicarboxylates.

25 Although diamides of themselves do thicken lubricating oils to the consistence of greases, it is known that such greases are of relatively low dropping point, that is, in general, in the region of 250° F. The presence of diamides in the grease thickening mixture of the present invention is detrimental to the dropping point.

30 The amate-dicarboxylate mixtures may be used in the preparation of greases according to this invention in amounts of 6% to 50% by weight, preferably 10% to 30%.

35 Examples of the greases prepared from the salt mixtures of the present invention are presented as follows:

*Example 1.—Preparation of lithium-N-hexadecyl adipamate-lithium adipate thickened grease*

40 A mixture of 58.5 grams (0.4 mol) of adipic acid and 500 ml. of 95% ethanol was heated to boiling in a 4 liter stainless steel beaker. To this mixture was added 72 grams (0.3 mol) of n-hexadecyl amine (Armeen 16D from Armour & Company) in 200 ml. of ethanol. The 45 ethanol solution of n-primary hexadecyl amine was added dropwise with rapid stirring while the whole reaction mixture was heated at reflux temperature. After all of the n-hexadecyl amine had been added, the ethanol was removed by evaporation.

50 The resulting solid reaction product was purified by heating the solid product to a temperature of 450° F., then pouring it directly into 1½ liters of water with rapid stirring, after which the slurry was heated to the boiling point of water, with stirring. After the slurry had been 55 cooled to 80° F., the solid was removed by filtration, then dried. This dried product was finely ground, dissolved in 500 ml. of boiling benzene, crystallized overnight, filtered and dried.

55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910

milled through a 200-mesh screen. The resulting grease was dark brown and smooth to the touch, and had a dropping point of 429° F., and an ASTM worked penetration of 287 at 78° F. (60 strokes).

*Example 2.—Preparation of grease thickened with lithium-N-hexadecyl dilinoleamide-lithium dilinoleate*

300 grams (1.5 moles) of dilinoleic acid<sup>(1)</sup> were heated to 300° F., after which 136 grams (0.5 mole) or Armeen HTD<sup>(2)</sup> were added dropwise during a period of 15 minutes. The reaction mixture was heated, with stirring, at a temperature range of 400° F. to 420° F. until all of the water of reaction had been removed. Upon cooling, the reaction product was a dark sticky solid having a neutralization number of 64.

A mixture of 15 grams of the above solid reaction product and 85 grams of a California solvent-refined naphthenic base oil having a viscosity of 450 SSU at 100° F. was charged to an 800 ml. Pyrex beaker. This mixture was heated, with stirring, to 200° F., then an aqueous solution of 1.44 grams of LiOH·H<sub>2</sub>O was added. The mixture was heated to a temperature of 390° F. After cooling, the product was a clear amber grease.

In the above examples of the grease preparations, the salts were prepared "in situ"; however, the salts may also be prepared as separate products, then dispersed in oils to form greases. The amic acids themselves may also be prepared directly in the oil.

Table I hereinbelow presents data on the use of amate-dicarboxylate mixtures as grease thickeners according to this invention. The thickening agents were prepared by reacting various primary amines with adipic acid, followed by reaction with a metal hydroxide. With the exception of greases 9 and 10, which respectively contained 24% and 14%, all of the greases contained 16%, by weight, of the thickening agent.

The various symbols used in Table I are explained as follows:

"HTD" refers to Armeen HTD, a product of Armour and Company, Chicago, Illinois, containing 25% n-hexadecylamine, 70% n-octadecylamine, and 5% n-octadecenylamine.

"T" refers to Armeen T, a product of Armour and Company, Chicago, Illinois, containing a mixture comprising 30% hexadecylamine, 25% octadecylamine and 45% hexadecenylamine. 85% of this mixture consists of n-primary amines.

"C" amine refers to Armeen "C," which contains 8% octylamine, 9% decylamine, 47% dodecylamine, 18% tetradecylamine, 8% hexadecylamine, 5% octadecylamine, and 5% octadecenylamine.

"TD" refers to Armeen TD, which is a purified product of the above Armeen "T." The "TD" product contains 30% n-primary hexadecylamine, 25% n-primary octadecylamine and 45% n-primary octadecenylamine.

"HT" refers to Armeen HT, which is a mixture of amines comprising 25% hexadecylamine, 70% octadecylamine and 5% octadecenylamine. 85% of this mixture consists of n-primary amines.

Base oil "A" was a California solvent-refined naphthenic base oil having a viscosity of 450 SSU at 100° F.

Base oil "B" was a California solvent-refined paraffinic base oil having a viscosity of 480 SSU at 100° F.

Base oil "C" was a di(2-ethylhexyl) sebacate.

Base oil "D" was a poly(methylphenyl) siloxane.

Base oil "E" was a California solvent-refined naphthenic base having a viscosity of 90 SSU at 210° F.

<sup>1</sup> This dilinoleic acid is essentially a dibasic acid of approximately 600 molecular weight of Emery Industries, Inc., Cincinnati, Ohio. It is prepared by the dimerization of linoleic acid. Although the product is essentially a dibasic acid, approximately 12% of trilinoleic acid (a tribasic acid) and 3% of linoleic acid (a monobasic acid) are present.

<sup>2</sup> Armeen HTD is a product of the Armour Company, Chicago, Illinois, and contains 25% of n-hexadecylamine, 70% of n-octadecylamine, and 5% of n-octadecenylamine. The mean molecular weight of this product is 264.

TABLE I

| Experiment No. | Reactants for Soap Preparation |                          |                 | Grease Properties      |                                   |          |
|----------------|--------------------------------|--------------------------|-----------------|------------------------|-----------------------------------|----------|
|                | n-primary amine                | Mole Acid/<br>Mole Amine | Metal Hydroxide | Dropping Point,<br>°F. | ASTM Penetrate<br>(Worked 78° F.) | Base Oil |
| 10             | hexyl                          | 2                        | Li              | 421                    | 360                               | A        |
| 2              | cyclohexyl                     | 4                        | Li              | 500+                   | 355                               | A        |
| 3              | HTD                            | 2                        | Na              | 486                    | 195                               | B        |
| 4              | HTD                            | 2                        | Al              | 431                    | 304                               | A        |
| 5              | phenyl                         | 4                        | Li              |                        |                                   | A        |
| 6              | octadecyl                      | 2                        | Li              | 474                    | 350                               | D        |
| 7              | T                              | 2                        | Li              | 500+                   | 284                               | A        |
| 8              | TD                             | 2                        | Li              | 500+                   | 360                               | A        |
| 9              | HT                             | 2                        | Li              | 500+                   | 282                               | B        |
| 10             | HT                             | 2                        | Li              | 500+                   | 285                               | E        |
| 11             | T                              | 2                        | Li              | 500+                   | 334                               | A        |
| 12             | C                              | 3                        | Li              | 500+                   | 313                               | A        |

When the amate-dicarboxylate grease thickening agents described herein are prepared from high molecular weight amines and/or high molecular weight dibasic acids, small amounts (e. g., less than 6%) of such amate-dicarboxylate mixtures can be used to thicken lubricating oils. Similarly, when amate-dicarboxylate mixtures are prepared from low molecular weight amines and/or dibasic acids, excellent lubricating oil thickening agents are obtained; that is, lubricating oils thickened to the consistency of extremely soft greases or greases having extremely low yield values. Such thickened lubricating oils may be used for filter elements, such as in air filter elements of diesel engines, air-conditioning units in general, etc.

As another embodiment of this invention, a dibasic acid salt may be added to an oil containing an amic acid salt; or a dibasic acid may be mixed with an amic acid before neutralization with a metal. For example, if in the original preparation of the amic acid-dibasic acid mixture, the mole ratio of dibasic acid to amine has a value of 1 or less than 1, additional dibasic acid may be incorporated into the amic acid thus prepared before neutralization with metal hydroxide, or additional dibasic acid salt may be incorporated into the oil prior to the grease preparation. The dibasic acid (or salt) added may or may not be the same as that used in the original preparation.

The necessity for the presence of dibasic acid salts in the grease thickening agents of this invention is illustrated in Example 3 hereinbelow.

*Example 3*

An amic acid-dibasic acid mixture (product A) was prepared from 219 grams (1.5 mols) of adipic acid and 311 grams (1 mol) of Armeen T (defined hereinabove). A portion of this mixture (which contained 2.68% nitrogen) was saponified with lithium hydroxide monohydrate and dispersed in a California solvent-refined oil, forming a grease having a dropping point of 435° F.

A second portion of the above amic acid-dibasic acid mixture was thoroughly agitated in hot water, separating the adipic acid from the amic acid. The amic acid (product B) contained 3.04% nitrogen. This amic acid was saponified with lithium hydroxide monohydrate and dispersed in a California solvent-refined oil, forming a grease having a dropping point of only 324° F.

25.6 grams of the above amic acid (product B) were mixed with 4.4 grams of adipic acid, and this mixture was saponified with lithium hydroxide monohydrate and dispersed in a California solvent-refined oil, forming a grease having a dropping point in excess of 500° F.

Although the grease thickening agents of this invention can be used in lubricating oils in amounts of 6% to 50%, by weight, 10% to 30% are preferred. In the formation of thickened lubricating oils useful for filter oils or for rustproofing agents, less than 6% may be used. That is, in lubricating oils thickened to less than grease consistency,

less than 6% of the thickening agents of this invention can be used.

In addition to the metal soap grease thickening agents of this invention, the grease composition may contain various additives, such as oxidation inhibitors, other thickening agents, gel modifiers, color correctors, extreme pressure agents, etc.

I claim:

1. A grease composition comprising a lubricating oil and a grease thickening agent in an amount sufficient to thicken said lubricating oil to the consistency of a grease, said thickening agent being prepared by reacting adipic acid with an amine containing from 12 to 18 carbon atoms, wherein the mol ratio of adipic acid to amine has a value from 1.5 to 5, then neutralizing the resulting adipic acid-amic acid mixture with an alkali metal hydroxide. 10

2. A grease composition comprising a lubricating oil and from 6% to 50%, by weight, of a grease thickening agent obtained by reacting adipic acid with n-octadecylamine, wherein the mol ratio of said adipic acid to said n-octadecylamine has a value from 1.5 to 5, forming a metal salt of said adipic acid-n-octadecyladipamate mixture by neutralizing said mixture with an alkali metal hydroxide. 20

3. A grease composition comprising a lubricating oil and from 6% to 50%, by weight, of a grease thickening agent obtained by reacting sebacic acid with n-octadecylamine, wherein the mol ratio of said sebacic acid to said n-octadecylamine has a value from 1.5 to 5, forming a metal salt of said sebacic acid-n-octadecyl-sebacamate mixture 25

30 by neutralizing said mixture with an alkali metal hydroxide.

4. A grease composition comprising a major proportion of a lubricating oil and a grease thickening agent in an amount sufficient to thicken said lubricating oil to the consistency of a grease, said thickening agent being obtained by reacting sebacic acid with an amine containing from 12 to 18 carbon atoms, wherein the mol ratio of sebacic acid to amine has a value of 1.5 to 5, neutralizing the resulting sebacic acid-amic acid mixture with an alkali metal hydroxide. 5

5. A grease composition comprising a lubricating oil and a grease thickening agent in an amount sufficient to thicken said lubricating oil to the consistency of a grease, said thickening agent being prepared by reacting a dibasic acid containing from 4-10 carbon atoms with an amine containing from 12-8 carbon atoms, wherein the mol ratio of dibasic acid to amine has a value from 1.5 to 5, then neutralizing the resulting dibasic acid-amic acid mixture with an alkali metal hydroxide. 15

6. The grease composition of claim 5 wherein the two carboxyl groups of said dibasic acid are attached as terminal groups to a polymethylene radical. 20

References Cited in the file of this patent

UNITED STATES PATENTS

|           |               |               |
|-----------|---------------|---------------|
| 1,937,463 | Nill          | Nov. 28, 1933 |
| 2,495,651 | Butcosk       | Jan. 24, 1950 |
| 2,594,286 | Bryant et al. | Apr. 29, 1952 |
| 2,604,449 | Bryant et al. | July 22, 1952 |